

# UNITED STATES PATENT OFFICE.

CHARLES ROBESON SQUIRE, OF NEW YORK, N. Y., ASSIGNOR OF ONE-HALF  
TO JAMES F. HOTCHKISS, OF PLAINFIELD, NEW JERSEY.

## TREATMENT OF ORES FOR AMALGAMATION.

SPECIFICATION forming part of Letters Patent No. 312,587, dated February 17, 1885.

Application filed April 10, 1883. Renewed December 10, 1884. (No specimens.)

*To all whom it may concern:*

Be it known that I, CHARLES ROBESON SQUIRE, of the city, county, and State of New York, have invented certain new and useful 5 Improvements in the Treatment of Ores for Amalgamation Containing the Precious Metals, of which the following is a specification.

This invention consists in a process of preparing the ores for perfect amalgamation.

10 My invention also consists in effecting a complete desulphurizing of the ores by a process at once efficient and simple, it having advantages over prior known processes in which soda-ash has been used either in combination 15 with the ore to facilitate its roasting or in combination with various elements, all intended to aid its own assumed insufficient action.

While the processes now in use free the 20 sulphur to a greater or lesser extent, none of them, so far as I am informed, prepare the gold for immediate amalgamation, for in the act of roasting the ores the gold becomes more or less coated with the oxide of iron, and in consequence passes over the plates and is lost. 25 My invention fully overcomes this difficulty and renders the gold free for instant amalgamation, as during the pulverization the metals are scoured and brightened, thus preventing the usual glaze of oxide of iron.

30 In conducting my improved process I use a mixture of two solutions. These are employed either before or after the ore has been roasted, as the different ores may require, either in a 35 bath alone of the mixed solutions or in an amalgamator with mercury. The solutions are as follows:

Solution No. 1: The residuum from the manufacture of muriatic (hydrochloric) acid, which 40 manufacture is effected by means of sulphuric acid on common salt. This residuum is sometimes called "salt-cake," and an analysis thereof is substantially as follows:

|                        | Parts. |
|------------------------|--------|
| Sulphate of soda ..... | 95     |
| Chloride of soda ..... | 2      |
| Sulphuric acid .....   | 2      |
| Magnesia, &c. ....     | 1      |
| Total .....            | 100    |

50 Solution No. 2: The residuum from the manu-

facture of nitric acid. This residuum is sometimes called "niter-cake," and its analysis is substantially as follows:

|                           | Parts. |
|---------------------------|--------|
| Sulphate of soda .....    | 75.90  |
| Free sulphuric acid ..... | 16.61  |
| Water .....               | 6.01   |
| Insoluble matter .....    | 1.29   |
| Total .....               | 99.81  |

60

The strength of the solutions must be determined by experience. Solution No. 1 may be used of, say, 22°, and No. 2, 38°, Baumé, subject to variation, as occasion may require. 65

If before or after the ore has been roasted it is treated with a mixture of solutions Nos. 1 and 2, either in a bath of the solutions alone or in an amalgamator with mercury, the solutions have a scouring effect upon the oxide of 70 iron and gold, by means of which the iron is removed and the gold left free to be taken up by the mercury. This action is partially chemical and partially due to the mechanical action of the pulverizer. It has been found 75 that the mercury cannot flour or float in amalgamating, either in this or any other process in the presence of the mixed solution which I have described.

The solutions may be used together in various proportions and of different strength, as experience may suggest, for different operations or qualities or grades of ores.

This process applies to all ores carrying gold or silver, and by its employment I have 85 in all cases obtained an amount running within eighty to ninety-five per cent. of fine assay.

I am aware that soda-ash has been employed either alone or in company with carbon and 90 other substances as a necessary addition to ores prior to and for the purpose of facilitating the roasting process, in combination with carbon, salt solution, and other materials in an atmosphere of steam; but I am not aware 95 that it has been used either alone or in combination with niter-cake, either before or after the heating of the ore indifferently to prepare the ore in addition to desulphurizing it for ready amalgamation.

I do not claim herein the use of either niter-cake or salt-cake separately, as such claims

100

are embodied in applications Nos. 101,519 and 101,520, filed July 21, 1883.

I claim as my invention—

1. The within-described process of preparing ores for amalgamation, which consists in subjecting the ore to a mixture of a solution of salt-cake and a solution of niter-cake, substantially as hereinbefore set forth.

2. The within-described process of desulphurizing ores, which consists in subjecting

them to a mixture of a solution of salt-cake and a solution of niter-cake, substantially as hereinbefore set forth.

In testimony whereof I have hereunto set my hand and seal this 9th day of April, A. D. 1883.

CHARLES ROBESON SQUIRE. [L. S.]

Witnesses:

JOHN G. MIDDLETON,  
JAMES F. HOTCHKISS.